

# United States Patent

[19]

Bomford

[11] 3,909,309

[45] Sept. 30, 1975

[54] **POST WORKING OF MECHANICALLY  
ALLOYED PRODUCTS**

[75] Inventor: **Michael James Bomford**, Bublikon,  
Switzerland

[73] Assignee: **The International Nickel Company,  
Inc.**, New York, N.Y.

[22] Filed: **Sept. 11, 1973**

[21] Appl. No.: **396,204**

[52] U.S. Cl..... **148/11.5 F**

[51] Int. Cl.<sup>2</sup>..... **B22F 1/00; B22F 3/14**

[58] Field of Search..... **148/11.5 F; 75/.5 BC**

[56] **References Cited**

UNITED STATES PATENTS

3,346,427 10/1967 Baldwin et al..... **148/11.5 F**

|           |         |                     |                   |
|-----------|---------|---------------------|-------------------|
| 3,494,807 | 2/1970  | Stuart et al.....   | <b>148/11.5 F</b> |
| 3,660,049 | 5/1972  | Benjamin.....       | <b>29/182.5</b>   |
| 3,746,581 | 7/1973  | Cairns et al.....   | <b>148/11.5 F</b> |
| 3,749,612 | 7/1973  | Benjamin et al..... | <b>148/11.5 F</b> |
| 3,776,704 | 12/1973 | Benjamin.....       | <b>75/.5 BC</b>   |
| 3,814,635 | 6/1974  | Cometto et al.....  | <b>148/11.5 R</b> |

*Primary Examiner*—W. Stallard

*Attorney, Agent, or Firm*—Raymond J. Kenny; Ewan  
C. MacQueen

[57]

## ABSTRACT

Special post extrusion working of mechanically alloyed superalloys dispersion-strengthened with an oxide of a lanthanide series metal results in improved stress-rupture properties.

**9 Claims, No Drawings**

## POST WORKING OF MECHANICALLY ALLOYED PRODUCTS

The present invention is addressed to mechanically alloyed dispersion-strengthened materials, particularly nickel-base superalloys containing a lanthanide metal oxide dispersoid.

"Mechanical alloying," described in U.S. Pat. Nos. 3,591,362 and 3,723,092 and incorporated herein by reference, involves, as is known, the dry and intensive milling of powders in high energy machines and under special conditions during which constituent powders are repeatedly fragmented and cold bonded by the continuous impacting action of attriting elements. This processing is continued for a period such that composite product powder particles of saturation, or at least substantial saturation, hardness are formed, the composition of which correspond to the percentages of the respective components in the original charge. By reason of this, the constituent powders become most intimately interdispersed at close interparticle spacings, the composite particles being exceptionally dense and homogeneous, and characterized by cohesive internal structures. A further attribute of this development is that it permits of precipitation hardening, dispersion strengthening and matrix stiffening to be brought together in one alloy, particularly the nickel and nickel-chromium superalloys.

By far and large, practically all thermomechanical processing of mechanically alloyed superalloy composite particles has been accomplished by virtue of extrusion, with improved extrusion parameters having been recently developed as set forth in copending U.S. Pat. application 131,761. As extrusion has dominated the thermomechanical processing scene, so yttria and thoria have received virtually exclusive attention as the dispersoids. However, since cost is always an important factor, other oxide dispersoids have been investigated and this has brought forth an unexpected problem.

When thoria or yttria are used as the dispersoid, a highly satisfactory level of stress-rupture properties can be consistently achieved. However, with lanthanide series metal oxides such as lanthana, ceria, didymia and the like, stress-rupture properties are often quite inferior. The complete theoretical mechanism which might explain this anomaly is not yet at hand, but an excess of fine grains is usually found subsequent to the conventional germinative grain growth heat treatment and this is considered responsible for the less attractive properties. In any case, it has been found that if mechanically alloyed superalloys dispersion hardened by one or more lanthanide metal oxides are hot worked as herein described subsequent to extrusion but prior to heat treatment, a high level of stress-rupture characteristics can nonetheless be obtained.

Generally speaking and in accordance herewith, the overall stress-rupture properties at elevated temperatures of mechanically alloyed superalloys, notably the nickel and/or cobalt-base compositions, dispersion-strengthened by an oxide of a lanthanide series metal are markedly enhanced by extruding a compact of the composite alloy particles and thereafter hot working (as by forging or hot rolling) the extruded product under correlated conditions of temperature and reduction such that upon germinative grain growth heat treatment a product is produced having a coarse, elongated grain structure, there being few, if any, fine grains.

In terms of the mechanical alloying process itself, the initial powder charge should be carried out to the point of at least "substantial saturation hardness", i.e., the level at which there is about at least a 50% difference between the base hardness of the alloy in the unworked condition and its saturated hardness in substantially the fully coldworked condition, this to provide mechanically alloyed powders of substantially homogeneous microstructure, such that upon examination of the structure of the powder at a magnification of, say, 250 diameters there is virtually no evidence of the starting material, the initial powder ingredients having been intimately united and interdispersed.

In the subsequent operations of extrusion (hot consolidation) of the composite powder and post-consolidation hot working, it is important that the working temperatures and reduction ratios be correlated to provide sufficiently worked consolidated bodies that can subsequently be heat treated to produce the desired coarse elongated grains. Underworked consolidated products generally result in small equiaxed grains when they are given the grain coarsening heat treatment while overworked consolidated products generally result in coarse equiaxed grains and/or cracking of the consolidated product during working. Working consolidated products at too low a temperature should be avoided to minimize the possibility of cracking during the working operation. It is accordingly important that the conditions of temperatures and reduction set forth herein be met.

Extrusion of the composite powder should be conducted at a temperature higher than about 1400°F., so to achieve substantially 100% density in the consolidated product. The composite powder is preferably consolidated by hot extruding at a temperature of about 1600°F. to 2100°F. at an extrusion ratio of about 4:1 to 50:1.

Post extrusion hot working can be carried out as by hot forging or hot rolling, it being generally preferred that the amount of hot working be greater for alloys containing lower amounts of dispersoid material and less for higher dispersoid contents. For example, a reduction of about 20 to about 80% at about 1600°F. can be used where the dispersoid content of the consolidated product is about 1 or 1½% or less, by volume, while about 10 to about 40% reduction at about 2000°F. can be used where the dispersoid content is about 3% or more, with a reduction of about 20 to 70% at 1800°F. being advantageous with dispersoid contents of about 1.5 to about 3%.

Post extrusion hot working or hot rolling should preferably be conducted over the temperature and reduction ranges shown in Table I below, where the consolidated products contain about 0.5 to about 5%, by volume, lanthanide metal oxide dispersoid material having an average particle size of about 50 Angstroms to about 600 Angstroms.

TABLE I

| Dispersoid                         | Working Operation | WORKING CONDITION               |                             |
|------------------------------------|-------------------|---------------------------------|-----------------------------|
|                                    |                   | Working Temp. (°F.) approx.     | Working Reduct. (approx.) % |
| La <sub>2</sub> O <sub>3</sub>     | hot forge         | 1550 to 2000<br>(1600 to 1900)* | 10 to 80<br>(20 to 60)*     |
|                                    | hot roll          | 1650 to 2000<br>(1650 to 1850)* | 25 to 60<br>(25 to 45)      |
| Di <sub>2</sub> O <sub>3</sub> (a) | hot forge         | 1700 to 2100<br>(1900 to 2100)  | 10 to 80<br>(20 to 60)*     |

TABLE I-Continued

| WORKING CONDITION |                   |                                 |                             |
|-------------------|-------------------|---------------------------------|-----------------------------|
| Dispersoid        | Working Operation | Working Temp. (°F.) approx.     | Working Reduct. (approx.) % |
| R.E.O.(b)         | hot roll          | 1700 to 2100<br>(1800 to 2050)* | 10 to 80<br>(20 to 60)*     |
|                   | hot forge         | 1600 to 2000<br>(1750 to 1900)* | 10 to 60<br>(15 to 45)*     |
|                   | hot roll          | 1700 to 2000<br>(1750 to 2000)* | 20 to 60<br>(25 to 45)*     |
|                   | hot forge         | 1700 to 2000<br>(1700 to 1850)* | 10 to 60<br>(15 to 40)*     |

\*Preferred

(a) Nominal comp.: 40-45% lanthana, 32-37% neodymia, 8-12% praeoedymia, balance oxides of other lanthanide metals.

(b) Nominal comp.: 24% lanthana, 48% ceria, 5% praeoedymia, 17% neodymia and balance essentially oxides of other lanthanide series metal.

Where stress-rupture properties at intermediate temperatures, e.g., 1400°F., are important, the extruded products should be hot worked according to Table II.

TABLE II

| WORKING CONDITION              |                   |                                 |                         |
|--------------------------------|-------------------|---------------------------------|-------------------------|
| Dispersoid                     | Working Operation | Working Temp. (°F.)             | Working Reduct. (%)     |
| La <sub>2</sub> O <sub>3</sub> | hot forge         | 1550 to 2000<br>(1600 to 1900)* | 10 to 80<br>(20 to 60)* |
|                                | hot roll          | 1650 to 2000<br>(1650 to 1850)* | 25 to 60<br>(40 to 60)* |
|                                | hot forge         | 1700 to 2100<br>(1900 to 2100)* | 10 to 80<br>(20 to 60)* |
|                                | hot roll          | 1700 to 2100<br>(1800 to 2100)* | 10 to 80<br>(20 to 60)* |
| R.E.O.                         | hot forge         | 1600 to 2000<br>(1750 to 1900)* | 10 to 60<br>(15 to 45)* |
|                                | hot roll          | 1600 to 2000<br>(1600 to 1900)* | 20 to 60<br>(25 to 50)* |

\*Preferred

The hot worked consolidated products described above are thereafter heated to attain coarse elongated grained products. A suitable temperature range is from about 2200°F. or higher, up to the incipient melting point of the alloy for periods of about ½ to 4 hours. The coarsened grains thus produced generally will have average dimensions of about 500 to 5000 microns in length and about 50 to 1000 microns in width, and are elongated in the direction or directions of working. It is important that the hot working operation always precede the grain coarsening heat treatment and it is desirable that the exposure of the consolidated product to elevated temperatures, e.g., 2150°F. or higher, prior to

hot working be minimal and preferably be avoided, to avoid impairing the producibility of coarse, elongated grains by the grain-coarsening heat treatment subsequent to hot working.

## EXAMPLE I

An 8.5 kg powder charge containing 6.42 kg of nickel having an average particle size of 5 µm, 1.7 kg of Cr having an average size of 50 µm, 1.3 kg of a Ni-8.5% Al-17% Ti master alloy with an average size of 50 µm, 0.02 kg of a Ni-29% Zr (master alloy) and .003 kg of a Ni-18% boron master alloy and 0.153 kg of lanthana having an average particle size of about 400 angstroms, prepared by calcining lanthanum oxalate at a temperature of 1300°F., was mechanically alloyed in a 10-gallon capacity attritor for a period of 17 hours at an impeller speed of 182 rpm, the attritor being provided with 390 pounds of +1/4 inch nickel pellets, which served as the attrition medium. Upon completion of the mechanical alloying, the minus 45 mesh fraction of the mechanically alloyed powder was packed in mild steel cans of 3 1/2 inch diameter and the cans were sealed and extruded at 1900°F. at ram speed of 0.5 linear feet per second to rectangular bars 5/8 by 1/8 inches in cross-sectional dimension, the extrusion reduction ratio being 16:1.

The consolidated alloy contained by weight, 20% chromium, 1.2% aluminum, 2.4% titanium, 0.07% zirconium, 0.007% boron, 2 1/4 volume % lanthana having an average particle size of about 400 Angstroms, the balance being essentially nickel. A portion of the as-extruded bar was heated at 2400°F. for 2 hours without any prior hot working, and the product exhibited fine grains. Upon aging and the testing at 1900°F., it was found that the stress-rupture life was virtually nil at 16,000 psi stress.

Pieces of the extruded bar were worked either by forging or rolling, at various elevated temperatures and various reductions (Tables III and IV), the reduction being applied to the 5/8 inch dimension except where stated otherwise. In the rolling procedure, the reduction per pass was about 15%.

The thus-hot worked pieces were given a grain coarsening heat treatment of 2400°F. for 2 hours and then were aged by heating at 1975°F. for 7 hours and at 1300°F. for 16 hours. Specimens from the grain coarsened-and-aged pieces were tested for stress-rupture properties at 1900°F. and 1400°F., the results being set out in Tables III and IV.

TABLE III

| Working Operation | 1900°F. Stress Rupture Properties<br>La <sub>2</sub> O <sub>3</sub> Dispersoid |                        |             |                 |       |      |
|-------------------|--------------------------------------------------------------------------------|------------------------|-------------|-----------------|-------|------|
|                   | Working Temperature<br>°F.                                                     | Working Reduction<br>% | Stress(psi) | Life<br>(hours) | % El. | % RA |
| Forging           | 1900                                                                           | 36                     | 17,000      | 309.4           | 0.8   | 0    |
|                   | 1800                                                                           | 45                     | 20,000      | 518.2           | 2.5   | 0    |
|                   | 1800                                                                           | 45                     | 16,000      | 67.1*           |       |      |
|                   |                                                                                |                        | 18,000      | 476.3**         | 3.7   | —    |
|                   | 1800                                                                           | 40.5                   | 20,000      | 826.0           | 2.5   | 3.0  |
|                   | 1800                                                                           | 40.5                   | 16,000      | 19.6*           |       |      |
|                   |                                                                                |                        | 18,000      | 274.1           | 2.5   | 9.9  |
|                   | 1800                                                                           | 36                     | 16,000      | 332.9*          |       |      |
|                   |                                                                                |                        | 18,000      | 276.2           | 1.25  | 0    |
|                   | 1800                                                                           | 36                     | 17,000      | 8.7             | 1.2   | 3.5  |
|                   | 1700                                                                           | 29.5                   | 17,000      | 316.9**         | 1.2   | —    |
|                   | 1700                                                                           | 29.5                   | 16,000      | 475.8*          |       |      |
|                   |                                                                                |                        | 18,000      | 126.7           | 2.5   | 0    |

TABLE III—Continued

| Working Operation | Working Temperature | 1900°F. Stress Rupture Properties<br>(La <sub>2</sub> O <sub>3</sub> Dispersoid) |        | Life<br>(hours) | % El. | % RA |
|-------------------|---------------------|----------------------------------------------------------------------------------|--------|-----------------|-------|------|
|                   |                     | °F.                                                                              | %      |                 |       |      |
| Rolling           | 1600                | 27.5                                                                             | 16,000 | 162.0*          |       |      |
|                   |                     |                                                                                  | 18,000 | 191.9**         | 2.5   | —    |
|                   | 1800                | 29.5                                                                             | 22,000 | 37.7            | 3.7   | 7.0  |
|                   | 1800                | 29.5                                                                             | 20,000 | 266.1           | 5.0   | 7.0  |
|                   | 1800                | 29.5                                                                             | 18,500 | 428.3           | 3.7   | 0    |
|                   | 1700                | 50.5                                                                             | 17,000 | 132.9           | 1.2   | 0    |

\*Specimen unbroken - stress raised

\*\*Specimen unbroken - test discontinued - grip or furnace failure.

TABLE IV

| Working Operation | Working Temperature<br>°F. | 1400°F. Stress Rupture Properties<br>(La <sub>2</sub> O <sub>3</sub> Dispersoid) |             | Life<br>(hours) | % El. | % RA |
|-------------------|----------------------------|----------------------------------------------------------------------------------|-------------|-----------------|-------|------|
|                   |                            | Working Reduction<br>%                                                           | Stress(psi) |                 |       |      |
| Forging           | 1900                       | 36                                                                               | 40,000      | 52.1            | 3.0   | 16.9 |
|                   | 1800                       | 36                                                                               | 40,000      | 34.3            | 5.0   | 14.0 |
|                   | 1800                       | 36                                                                               | 35,000      | 717.0*          |       |      |
|                   |                            |                                                                                  | 37,500      | 73.8            | 3.8   | 8.5  |
|                   | 1800                       | 42                                                                               | 40,000      | 12.5            | 8.7   | 25.7 |
|                   | 1700                       | 29.5                                                                             | 40,000      | 19.4            | 8.5   | 20.6 |
|                   | 1700                       | 29.5                                                                             | 35,000      | 425.9           | 2.5   | 7.7  |
|                   | 1600                       | 27.5                                                                             | 40,000      | 6.3             | 7.5   | 13.9 |
|                   | 1800                       | 29.5                                                                             | 40,000      | 6.4             | 13.7  | 28.0 |
|                   | 1700                       | 50.5                                                                             | 40,000      | 15.4            | 5.0   | 7.8  |

\*Specimen unbroken - stress raised.

From Table III, it can be seen that forging the lanthana-containing extrusions in the temperature range of 1600°F. to 1900°F. with reductions of about 27.5 to 45% and the grain coarsening at 2400°F. provides 100-hour stress-rupture lives at 1900°F. at stresses considerably greater than 17,000 psi, and that forging at 1800°F. to reductions of 40.5 to 45% and grain coarsening provides 100-hour stress-rupture lives at stresses significantly higher than 20,000 psi at 1900°F. These data compare well with the results obtained with respect to the as-extruded bar. Rolling the lanthana-containing alloy at 1700°F. to 1800°F. to reduce it by about 29.5 to about 50.5% and then grain coarsening at 2400°F. also provided 100 hour stress-rupture lives at 1900°F. at stresses higher than 17,000 psi as seen from Table III. Rolling the lanthana-containing consolidated product at a temperature on the order of about 1800°F. to achieve reductions on the order of 29.5% provided very good 1900°F. stress-rupture properties at a stress of 20,000 psi and even 22,000 psi, so that rolling under such conditions and subsequent grain coarsening can provide, in such consolidated products, a 100-hour life at 1900°F. at an applied stress of about 21,000 psi. The 1400°F. stress-rupture properties (Table IV) were generally good.

Metallographic examination of grain-coarsened pieces after the 2400°F. grain coarsening treatment, revealed grains having average dimensions of about 1000 microns in length and about 80 microns in width. The grain structure was substantially uniform and no fine-grained areas were evident.

## EXAMPLE II

An alloy similar in composition to that in Example I but having 2 1/4% of a dispersoid mixture (herein "refractory oxide mixture") comprising, by weight, 25% lanthana, 48% ceria, 17% neodymia, 5% praseodymia and the balance essentially oxides of other lanthanide series metals (average particle size of about 350 Angstroms), was mechanically alloyed in the manner given in Example I, except the processing time was 20 hours. The minus 45 mesh fraction was sealed in mild steel cans and extruded at 1900°F. at a reduction ratio of 16:1 to provide bar extrusions having a rectangular cross section of 5/8 × 15/16-inch dimensions.

One piece of the extruded bar was annealed at 2400°F. for 2 hours without prior hot working but no grain coarsening took place, this piece exhibiting a zero stress-rupture life at 1900°F. and a stress of 16,000 psi. Other pieces were forged unidirectionally over the ranges of temperatures and reductions shown in Table V and then annealed at 2400°F. for 2 hours to achieve grain coarsening, after which the grain-coarsened pieces were aged by heating at 1975°F. for 7 hours and then at 1300°F. for 16 hours. The thus-produced pieces were then tested for 1400°F. stress rupture properties, results being shown in Table V. Specimens that were also tested at 1900°F. at stresses of 16,000 and 18,000 psi exhibited lives of 703.8 and 130.9 hours, respectively, indicating the desirable elevated temperature properties obtainable with the present invention.

TABLE V

| Working Operation | Working Temperature<br>°F. | 1400°F. Stress Rupture Properties |                     |              |              |       |
|-------------------|----------------------------|-----------------------------------|---------------------|--------------|--------------|-------|
|                   |                            | R.E.O. Dispersoid                 | Working Reduction % | Stress (psi) | Life (hours) | % El. |
| Forging           | 2000                       | 39                                | 40,000              | 135.6        | 2.5          | 7.0   |
|                   | 1900                       | 29.5                              | 40,000              | 127.8        | 2.5          | 8.8   |
|                   | 1900                       | 29.5                              | 45,000              | 41.8         | 3.7          | 8.7   |
|                   | 1800                       | 37.5                              | 40,000              | 51.5         | 2.5          | 0.8   |
|                   | 1800                       | 37.5                              | 45,000              | 28.7         | 1.25         | 0     |
|                   | 1800                       | 32.5                              | 40,000              | 47.1         | 1.2          | 0     |
|                   | 1800                       | 22                                | 40,000              | 263.9        | 6.2          | 10.0  |
|                   | 1800                       | 29.5                              | 40,000              | 84.6         | 1.2          | 10.0  |
| Rolling           | 1700                       | 50                                | 40,000              | 17.8         | 7.5          | —     |

### EXAMPLE III

A mechanically alloyed powder having a nominal composition similar to that in Example I except that the dispersoid comprised about 2½ inch volume % didymium

tions shown in Table VI and then grain coarsened by heating at 2400°F. for 2 hours and stress-rupture tested at 1400°F. From the stress-rupture test results given in Table VI, it can be seen that satisfactory intermediate temperature range properties were obtained.

TABLE VI

| Working Operation | Working Temperature<br>°F. | 1400°F. Stress Rupture Properties<br>( $\text{Di}_2\text{O}_3$ Dispersoid) |             |       |      | Life<br>(hours) | % El. | % RA |
|-------------------|----------------------------|----------------------------------------------------------------------------|-------------|-------|------|-----------------|-------|------|
|                   |                            | Working Reduction<br>%                                                     | Stress(psi) |       |      |                 |       |      |
| Forging           | 2000                       | 46.5                                                                       | 40,000      | 420.5 | 5.0  | 12.5            |       |      |
|                   | 1900                       | 46                                                                         | 40,000      | 117.6 | 2.5  | 7.0             |       |      |
|                   | 1900                       | 46                                                                         | 45,000      | 52.0  | 3.8  | 5.8             |       |      |
|                   | 1800                       | 34.5                                                                       | 40,000      | 274.8 | 2.5  | 7.8             |       |      |
|                   | 1800                       | 34.5                                                                       | 45,000      | 52.7  | 2.5  | 5.8             |       |      |
|                   | 1800                       | 29.5                                                                       | 40,000      | 253.5 | 5.0  | 12.7            |       |      |
|                   | 1700                       | 33                                                                         | 40,000      | 98.3  | 1.2  | 1.5             |       |      |
|                   | 1700                       | 33                                                                         | 40,000      | 24.6  | 1.25 | 0               |       |      |
|                   | 1700                       | 33                                                                         | 45,000      | 33.3  | 0.8  | 1.4             |       |      |
|                   | 1800                       | 29.5                                                                       | 40,000      | 132.9 | 8.7  | 18.0            |       |      |
| Rolling           | 1800                       | 29.5                                                                       | 45,000      | 40.9  | 6.2  | 4.0             |       |      |
|                   | 1700                       | 51                                                                         | 40,000      | 4.3   | 1.2  | —               |       |      |

(153 grams, avg. particle size of 350 Angstroms) was produced in the manner described in Example I, except the mechanical alloying time was 20 hours. The minus 45 mesh fraction of the powder was extruded at 1900°F. with a 16:1 reduction ratio to produce  $\frac{5}{8}$  by  $\frac{15}{16}$  inch rectangular cross-section bar. A piece of this bar was annealed in the as-extruded condition at 2400°F. for 2 hours in an attempt to produce coarse elongated grains. Again, as excess of fine grains was found.

Other pieces of the bar were forged unidirectionally at, respectively, 1900°F. and 2000°F. to provide respective working reductions of about 46%. The thus-worked pieces were then heated at 2400°F. for 2 hours, which resulted in coarse elongated grains having average dimensions of about 100 microns wide and about 600 microns long, after which they were tested for stress-rupture properties at 1900°F. The pieces worked at 2000°F. were tested at stresses of 16,000 and 18,000 psi and had lives of 326.4 and 35.3 hours, respectively, while those worked at 1900°F. were tested at stresses of 15,000 and 16,000 psi and had lives of 233.0 and 24.1 hours, respectively.

Pieces of other extrusions having the same composition and produced in the same manner as the extruded bar just described were forged over the temperature range of 1700°F. to 2000°F. to provide reductions over the range of about 29.5 to 46.5% as indicated in Table VI, after which they were grain coarsened by heating at 2400°F. for 2 hours and then stress-rupture tested at 1400°F. Other such pieces were rolled under the condi-

40 In this instance 2½ volume % ceria was used as the dispersoid, the composition otherwise being similar to that in Example I. The mechanically alloyed powder was canned and extruded as described in Example I, after which various pieces of the extrusion were formed 45 at temperatures and reductions given in Table VII. The hot forged pieces were then grain coarsened by heating at 2400°F., the results being given in Table VII, from which table it can be seen that desirable elevated temperature properties were produced.

TABLE VII

| 1900°F. Stress Rupture Properties<br>(CeO <sub>2</sub> Dispersoid) |                             |                 |                 |       |      |  |
|--------------------------------------------------------------------|-----------------------------|-----------------|-----------------|-------|------|--|
| Forging<br>Temperature<br>(°F.)                                    | Forging<br>Reduction<br>(%) | Stress<br>(psi) | Life<br>(hours) | % El. | % RA |  |
| 1800                                                               | 39                          | 16,000          | 20.1            | 1.25  | 1.4  |  |
| 1700                                                               | 18                          | 16,000          | 44.2            | 3.8   | 2.9  |  |
| 1700                                                               | 18                          | 15,000          | 64.4            | 2.5   | 10.6 |  |

Alloys that can be processed in accordance with the instant invention include those containing up to about 65% chromium, up to about 8% aluminum, up to about 65 8% titanium, up to about 40% molybdenum, up to 40% tungsten, up to about 20% columbium, up to about 40% tantalum, up to about 5% vanadium, up to about 15% manganese, up to about 0.5% magnesium, up to about 2% carbon, up to about 3% silicon, up to about

1% boron, up to 2% zirconium, up to about 6% hafnium, up to about 40% iron, up to about 10% or more by volume of a dispersoid material comprising an oxide of lanthanide series metal, and the balance essentially nickel and/or cobalt.

It is generally preferred that the mechanically alloyed powder charge contain, by weight, about 5 to 35% chromium, at least one metal from the group of aluminum and titanium in a total amount of at least about 0.5 and up to about 13%, e.g., 0.5 to 6.5% of either or both aluminum and titanium, up to about 15% molybdenum up to about 20% tungsten, up to about 10% columbium, up to about 10% tantalum, up to about 3% vanadium, up to about 2% manganese, up to about 2% silicon, up to about 0.75% carbon, up to about 0.1% boron, up to 1% zirconium, up to about 0.2% magnesium, up to about 35% iron and about 1 to 3%, e.g., 1.75% to about 2.5%, by volume, of dispersoid material comprising an oxide of lanthanide series metal. It is preferred that the dispersoid particles have an average particle diameter of about 20 to 2000 Angstroms, more preferably, about 50 to about 1000 Angstroms.

Although the invention has been described in connection with preferred embodiments, modifications may be resorted to without departing from the spirit and scope of the invention, as those skilled in the art will readily understand. Such are considered within the purview and scope of the invention and appended claims.

I claim:

1. A process for achieving enhanced stress-rupture characteristics at elevated temperatures in respect of a mechanically alloyed superalloy composition containing as a dispersoid an oxide of a lanthanide series metal, whereby the alloy is capable of developing a desired structure having coarse elongated grains upon germinative grain growth treatment, which comprises hot consolidating a charge of such mechanically alloyed composite superalloy powder particles and thereafter hot working the resulting hot consolidated product, the temperature of hot working and amounts of reduction being correlated such that (a) the formation of small equiaxed grains upon grain coarsening heat treatment is minimized, and (b) the formation of coarse equiaxed grains and/or cracking of the consolidated product during the hot working operation is minimized, whereby coarse elongated grains result upon subsequent heating of the shape at germinative grain growth temperature.

2. A process in accordance with claim 1 in which the lanthanide metal series oxide dispersoid is of the group lanthana, didymia, rare earth oxide and ceria, the lanthana, didymia, rare earth oxides being respectively either hot forged or hot rolled within the combination of hot working temperature range and hot working reduction range given below.

-Continued

| Dispersoid     | Working Operation | Working Temp. (°F.) approx.    | Working Reduct. (approx.) % |
|----------------|-------------------|--------------------------------|-----------------------------|
| 5<br>R.E.O.(b) | hot forge         | 1600 to 2000<br>(1750 to 1900) | 10 to 60<br>(15 to 45)      |
|                | hot roll          | 1700 to 2000<br>(1750 to 2000) | 20 to 60<br>(25 to 45)      |
|                | hot forge         | 1700 to 2000<br>(1700 to 1850) | 10 to 60<br>(15 to 40)      |

10

3. A process in accordance with claim 2 in which the hot forging or hot rolling operation is conducted in accordance with the following:

| Dispersoid                           | Working Operation | Working Temp. (°F.)            | Working Reduct. (%)    |
|--------------------------------------|-------------------|--------------------------------|------------------------|
| 15<br>La <sub>2</sub> O <sub>3</sub> | hot forge         | 1550 to 2000<br>(1600 to 1900) | 10 to 80<br>(20 to 60) |
|                                      | hot roll          | 1650 to 2000<br>(1650 to 1850) | 25 to 60<br>(40 to 60) |
| 20<br>Dy <sub>2</sub> O <sub>3</sub> | hot forge         | 1700 to 2100<br>(1900 to 2100) | 10 to 80<br>(20 to 60) |
|                                      | hot roll          | 1700 to 2100<br>(1800 to 2100) | 10 to 80<br>(20 to 60) |
|                                      | hot forge         | 1600 to 2000<br>(1750 to 1900) | 10 to 60<br>(15 to 45) |
| R.E.O.                               | hot roll          | 1600 to 2000<br>(1600 to 1900) | 20 to 60<br>(25 to 50) |

25

4. A process in accordance with claim 2 in which the dispersoid material is present in an amount of up to about 10% by volume.

30 5. A process in accordance with claim 2 in which the dispersoid material is present in an amount of about 1 to 3% by volume.

35 6. A process in accordance with claim 1 in which the dispersion-strengthened mechanically alloyed superalloy is of a composition containing up to 65% chromium, up to about 8% aluminum, up to about 8% titanium, up to about 40% molybdenum, up to 40% tungsten, up to about 20% columbium, up to about 40% tantalum, up to about 5% vanadium, up to about 15% manganese, up to about 0.5% magnesium, up to about 2% carbon, up to about 3% silicon, up to about 1% boron, up to 2% zirconium, up to about 6% hafnium, up to about 40% iron, up to about 10% or more by volume of a dispersoid material comprising an oxide of lanthanide series metal, and the balance essentially nickel and/or cobalt.

40 7. A process in accordance with claim 1 in which the dispersion-strengthened mechanically alloyed superalloy is of a composition containing about 5% to about 35% chromium, about 0.5% to about 13% of metal from the group of aluminum and titanium, up to about 15% molybdenum, up to about 20% tungsten, up to about 10% columbium, up to about 10% tantalum, up to about 3% vanadium, up to about 2% manganese, up to about 2% silicon, up to about 0.75% carbon, up to about 0.1% boron, up to 1% zirconium, up to about 0.2% magnesium, up to about 35% iron, and about 1 to 3% by volume of dispersoid material.

45 8. A process in accordance with claim 2 in which the hot worked product is heated at a temperature of from about 2200°F. to below the incipient melting point of the alloy, whereby a microstructure is obtained having coarse elongated grains and few, if any, fine grains.

50 9. A process in accordance with claim 2 in which the dispersoid is of an average particle size of about 150 to about 600 Angstroms.

| Dispersoid                         | Working Operation | Working Temp. (°F.) approx.    | Working Reduct. (approx.) % |
|------------------------------------|-------------------|--------------------------------|-----------------------------|
| La <sub>2</sub> O <sub>3</sub>     | hot forge         | 1550 to 2000<br>(1600 to 1900) | 10 to 80<br>(20 to 60)      |
|                                    | hot roll          | 1650 to 2000<br>(1650 to 1850) | 25 to 60<br>(40 to 60)      |
| Dy <sub>2</sub> O <sub>3</sub> (a) | hot forge         | 1700 to 2100<br>(1900 to 2100) | 10 to 80<br>(20 to 60)      |
|                                    | hot roll          | 1700 to 2100<br>(1800 to 2050) | 10 to 80<br>(20 to 60)      |

\* \* \* \* \*